



US008712304B2

(12) **United States Patent**  
**Wu et al.**

(10) **Patent No.:** **US 8,712,304 B2**  
(45) **Date of Patent:** **Apr. 29, 2014**

(54) **FUSER MEMBER**

(75) Inventors: **Jin Wu**, Pittsford, NY (US); **Lanhui Zhang**, Webster, NY (US); **Lin Ma**, Pittsford, NY (US); **Jonathan H. Herko**, Walworth, NY (US)

(73) Assignee: **Xerox Corporation**, Norwalk, CT (US)

(\*) Notice: Subject to any disclaimer, the term of this patent is extended or adjusted under 35 U.S.C. 154(b) by 103 days.

(21) Appl. No.: **13/442,240**

(22) Filed: **Apr. 9, 2012**

(65) **Prior Publication Data**

US 2013/0266356 A1 Oct. 10, 2013

(51) **Int. Cl.**

**G03G 15/20** (2006.01)

(52) **U.S. Cl.**

USPC ..... 399/333; 399/307; 399/328; 399/329;  
430/124.32

(58) **Field of Classification Search**

USPC ..... 399/333, 329, 328, 330, 307;  
430/124.1, 124.11, 124.3, 124.32

See application file for complete search history.

(56) **References Cited**

**U.S. PATENT DOCUMENTS**

|                   |         |                   |           |
|-------------------|---------|-------------------|-----------|
| 4,585,829 A *     | 4/1986  | Kuo et al. ....   | 524/714   |
| 8,465,838 B2 *    | 6/2013  | Wu .....          | 399/333 X |
| 2006/0194011 A1 * | 8/2006  | Ito .....         | 428/35.7  |
| 2006/0275063 A1 * | 12/2006 | Blair et al. .... | 399/333   |
| 2012/0049123 A1 * | 3/2012  | Wu .....          | 252/500   |
| 2012/0052306 A1 * | 3/2012  | Wu et al. ....    | 428/421   |
| 2012/0076931 A1 * | 3/2012  | Wu .....          | 399/333 X |
| 2012/0148851 A1 * | 6/2012  | Wu .....          | 428/447   |
| 2012/0202078 A1 * | 8/2012  | Wu .....          | 428/447   |
| 2012/0231258 A1 * | 9/2012  | Wu .....          | 428/323   |
| 2012/0244345 A1 * | 9/2012  | Wu .....          | 428/337   |
| 2012/0244463 A1 * | 9/2012  | Wu et al. ....    | 430/84    |
| 2012/0261621 A1 * | 10/2012 | Wu .....          | 252/501.1 |

\* cited by examiner

*Primary Examiner* — Sophia S Chen

(74) *Attorney, Agent, or Firm* — Hoffman Warnick LLC

(57) **ABSTRACT**

The present teachings provide a fuser member. The fuser member includes a substrate layer having a polyimide polymer and a fluoro acid. A method of manufacturing a fuser member is also described.

**19 Claims, 3 Drawing Sheets**





FIG. 1



FIG. 2A



FIG. 2B



**1**  
**FUSER MEMBER**

BACKGROUND

1. Field of Use

This disclosure is generally directed to fuser members useful in electrophotographic imaging apparatuses, including digital, image on image, and the like. In addition, the fuser member described herein can also be used in a transfix apparatus in a solid ink jet printing machine.

2. Background

Centrifugal molding is used to obtain seamless polyimide belts useful as fuser members. Typically, a thin fluorine or silicone release layer is applied to the inner surface of a rigid cylindrical mandrel. A polyimide coating is applied to the inner surface of the mandrel containing the release layer. The polyimide is cured and then released from the mandrel.

There are drawbacks to this process. The length of the polyimide belt is determined by the size of the mandrel. The requirement of a release layer on the inner surface of the mandrel is an additional process step. For fuser belts manufactured in this manner the cost is expensive. There is a need to reduce the manufacturing cost.

In addition, a polyimide fuser belt requires a modulus that is greater than 4,000 MPa. It is a characteristic that the onset decomposition temperature be greater than 400° C. Such requirements, along with reduced cost of manufacturing are desirable.

SUMMARY

According to an embodiment, a fuser member is provided. The fuser member includes a substrate layer comprising a polyimide polymer and a fluoro acid.

According to another embodiment, there is described a fuser member including a substrate layer comprising a polyimide polymer and a fluoro acid having the structure selected from the group consisting of  $\text{HOOC}(\text{CF}_2)_n\text{COOH}$ , and  $\text{C}_n\text{F}_{2n+1}\text{COOH}$  wherein n is from 2 to 18. The fuser member includes an intermediate layer, disposed on the substrate layer comprising a material selected from the group consisting of silicone and fluoroelastomer. The fuser member includes a release layer, disposed on the intermediate layer comprising a fluoropolymer.

According to another embodiment, there is described a fuser member comprising a substrate layer including a polyimide polymer and a fluoro acid selected from the group consisting of  $\text{HOOC}(\text{CF}_2)_n\text{COOH}$  and  $\text{C}_n\text{F}_{2n+1}\text{COOH}$ , wherein n is from 2 to 18. The substrate layer has a modulus of from about 4,000 MPa to about 10,000 MPa and an onset decomposition temperature of about 590° C.

BRIEF DESCRIPTION OF THE DRAWINGS

The accompanying drawings, which are incorporated in and constitute a part of this specification, illustrate several embodiments of the present teachings and together with the description, serve to explain the principles of the present teachings.

FIG. 1 depicts an exemplary fuser member having a belt substrate in accordance with the present teachings.

FIGS. 2A-2B depict exemplary fusing configurations using the fuser member shown in FIG. 1 in accordance with the present teachings.

FIG. 3 depicts a fuser configuration using a transfix apparatus.

**2**

FIG. 4 depicts a tensioning of a fusing member for final curing.

It should be noted that some details of the FIGS. have been simplified and are drawn to facilitate understanding of the embodiments rather than to maintain strict structural accuracy, detail, and scale.

DESCRIPTION OF THE EMBODIMENTS

Reference will now be made in detail to embodiments of the present teachings, examples of which are illustrated in the accompanying drawings. Wherever possible, the same reference numbers will be used throughout the drawings to refer to the same or like parts.

In the following description, reference is made to the accompanying drawings that form a part thereof, and in which is shown by way of illustration specific exemplary embodiments in which the present teachings may be practiced. These embodiments are described in sufficient detail to enable those skilled in the art to practice the present teachings and it is to be understood that other embodiments may be utilized and that changes may be made without departing from the scope of the present teachings. The following description is, therefore, merely exemplary.

Furthermore, to the extent that the terms "including", "includes", "having", "has", "with", or variants thereof are used in either the detailed description and the claims, such terms are intended to be inclusive in a manner similar to the term "comprising." The term "at least one of" is used to mean that one or more of the listed items can be selected.

Notwithstanding that the numerical ranges and parameters setting forth the broad scope of the invention are approximations, the numerical values set forth in the specific examples are reported as precisely as possible. Any numerical value, however, inherently contains certain errors necessarily resulting from the standard deviation found in their respective testing measurements. Moreover, all ranges disclosed herein are to be understood to encompass any and all sub-ranges subsumed therein. For example, a range of "less than 10" can include any and all sub-ranges between (and including) the minimum value of zero and the maximum value of 10, that is, any and all sub-ranges having a minimum value of equal to or greater than zero and a maximum value of equal to or less than 10, e.g., 1 to 5. In certain cases, the numerical values as stated for the parameter can take on negative values. In this case, the example value of range stated as "less than 10" can assume negative values, e.g. -1, -2, -3, -10, -20, -30, etc.

The fuser or fixing member can include a substrate having one or more functional intermediate layers formed thereon. The substrate described herein includes a belt. The one or more intermediate layers include cushioning layers and release layers. Such fuser member can be used as an oil-less fusing member for high speed, high quality electrophotographic printing to ensure and maintain a good toner release from the fused toner image on an image supporting material (e.g., a paper sheet), and further assist paper stripping.

In various embodiments, the fuser member can include, for example, a substrate, with one or more functional intermediate layers formed thereon. The substrate can be formed in various shapes, such as a belt, or a film, using suitable materials that are non-conductive or conductive depending on a specific configuration, for example, as shown in FIG. 1.

In FIG. 1, an exemplary embodiment of a fusing or transfix member 200 can include a belt substrate 210 with one or more functional intermediate layers, e.g., 220 and an outer surface layer 230 formed thereon. The outer surface layer 230 is also

referred to as a release layer. The belt substrate **210** is described further and is made of a polyimide polymer and a fluoro acid.

#### Functional Intermediate Layer

Examples of materials used for the functional intermediate layer **220** (also referred to as cushioning layer or intermediate layer) include fluorosilicones, silicone rubbers such as room temperature vulcanization (RTV) silicone rubbers, high temperature vulcanization (HTV) silicone rubbers, and low temperature vulcanization (LTV) silicone rubbers. These rubbers are known and readily available commercially, such as SILASTIC® 735 black RTV and SILASTIC® 732 RTV, both from Dow Corning; 106 RTV Silicone Rubber and 90 RTV Silicone Rubber, both from General Electric; and JCR6115CLEAR HTV and SE4705U HTV silicone rubbers from Dow Corning Toray Silicones. Other suitable silicone materials include siloxanes (such as polydimethylsiloxanes); fluorosilicones such as Silicone Rubber **552**, available from Sampson Coatings, Richmond, Va.; liquid silicone rubbers such as vinyl crosslinked heat curable rubbers or silanol room temperature crosslinked materials; and the like. Another specific example is Dow Corning Sylgard 182. Commercially available LSR rubbers include Dow Corning Q3-6395, Q3-6396, SILASTIC® 590 LSR, SILASTIC® 591 LSR, SILASTIC® 595 LSR, SILASTIC® 596 LSR, and SILASTIC® 598 LSR from Dow Corning. The functional layers provide elasticity and can be mixed with inorganic particles, for example SiC or Al<sub>2</sub>O<sub>3</sub>, as required.

Other examples of the materials suitable for use as functional intermediate layer **220** also include fluoroelastomers. Fluoroelastomers are from the class of 1) copolymers of two of vinylidenefluoride, hexafluoropropylene, and tetrafluoroethylene; 2) terpolymers of vinylidenefluoride, hexafluoropropylene, and tetrafluoroethylene; and 3) tetrapolymers of vinylidenefluoride, hexafluoropropylene, tetrafluoroethylene, and a cure site monomer. These fluoroelastomers are known commercially under various designations such as VITON A®, VITON B®, VITON E®, VITON E 60C®, VITON E430®, VITON 910®, VITON GH®; VITON GF®; and VITON ETP®. The VITON® designation is a trademark of E.I. DuPont de Nemours, Inc. The cure site monomer can be 4-bromoperfluorobutene-1,1,1-dihydro-4-bromoperfluorobutene-1,3-bromoperfluoropropene-1,1,1-dihydro-3-bromoperfluoropropene-1, or any other suitable, known cure site monomer, such as those commercially available from DuPont. Other commercially available fluoropolymers include FLUOREL 2170®, FLUOREL 2174®, FLUOREL 2176®, FLUOREL 2177® and FLUOREL LVS 76®, FLUOREL® being a registered trademark of 3M Company. Additional commercially available materials include AFLAST™ a poly(propylene-tetrafluoroethylene), and FLUOREL IIR® (LII900) a poly(propylene-tetrafluoroethylene-vinylidenefluoride), both also available from 3M Company, as well as the Tecnoflons identified as FOR-60KIR®, FOR-LHF® NMR® FOR-THF®, FOR-TFS® TH® NH®, P757 TNS®, T439 PL958® BR9151® and TN505, available from Ausimont.

Examples of three known fluoroelastomers are (1) a class of copolymers of two of vinylidenefluoride, hexafluoropropylene, and tetrafluoroethylene, such as those known commercially as VITON A®; (2) a class of terpolymers of vinylidenefluoride, hexafluoropropylene, and tetrafluoroethylene known commercially as VITON B®; and (3) a class of tetrapolymers of vinylidenefluoride, hexafluoropropylene, tetrafluoroethylene, and cure site monomer known commercially as VITON GH® or VITON GF®.

The fluoroelastomers VITON GH® and VITON GF® have relatively low amounts of vinylidenefluoride. The VITON GF® and VITON GH® have about 35 weight percent of vinylidenefluoride, about 34 weight percent of hexafluoropropylene, and about 29 weight percent of tetrafluoroethylene, with about 2 weight percent cure site monomer.

The thickness of the functional intermediate layer **220** is from about 30 microns to about 1,000 microns, or from about 100 microns to about 800 microns, or from about 150 to about 500 microns.

#### Release Layer

An exemplary embodiment of a release layer **230** includes fluoropolymer particles. Fluoropolymer particles suitable for use in the formulation described herein include fluorine-containing polymers. These polymers include fluoropolymers comprising a monomeric repeat unit that is selected from the group consisting of vinylidene fluoride, hexafluoropropylene, tetrafluoroethylene, perfluoroalkylvinylether, and mixtures thereof. The fluoropolymers may include linear or branched polymers, and cross-linked fluoroelastomers. Examples of fluoropolymer include polytetrafluoroethylene (PTFE); perfluoroalkoxy polymer resin (PFA); copolymer of tetrafluoroethylene (TFE) and hexafluoropropylene (HFP); copolymers of hexafluoropropylene (HFP) and vinylidene fluoride (VDF or VF2); terpolymers of tetrafluoroethylene (TFE), vinylidene fluoride (VDF), and hexafluoropropylene (HFP); and tetrapolymers of tetrafluoroethylene (TFE), vinylidene fluoride (VF2), and hexafluoropropylene (HFP), and mixtures thereof. The fluoropolymer particles provide chemical and thermal stability and have a low surface energy. The fluoropolymer particles have a melting temperature of from about 255° C. to about 360° C. or from about 280° C. to about 330° C. These particles are melted to form the release layer.

For the fuser member **200**, the thickness of the outer surface layer or release layer **230** can be from about 10 microns to about 100 microns, or from about 20 microns to about 80 microns, or from about 40 microns to about 60 microns.

#### Adhesive Layer(s)

Optionally, any known and available suitable adhesive layer, also referred to as a primer layer, may be positioned between the release layer **230**, the functional intermediate layer **220** and the substrate **210**. Examples of suitable adhesives include silanes such as amino silanes (such as, for example, HV Primer 10 from Dow Corning), titanates, zirconates, aluminates, and the like, and mixtures thereof. In an embodiment, an adhesive in from about 0.001 percent to about 10 percent solution can be wiped on the substrate. The adhesive layer can be coated on the substrate, or on the outer layer, to a thickness of from about 2 nanometers to about 2,000 nanometers, or from about 2 nanometers to about 500 nanometers. The adhesive can be coated by any suitable known technique, including spray coating or wiping.

FIGS. 2A and 2B depict an exemplary fusing configuration for the fusing process in accordance with the present teachings. It should be readily apparent to one of ordinary skill in the art that the fusing configurations **300B** and **400B** depicted in FIGS. 2A-2B, respectively, represent generalized schematic illustrations and that other members/layers/substrates/configurations can be added or existing members/layers/substrates/configurations can be removed or modified. Although an electrophotographic printer is described herein, the disclosed apparatus and method can be applied to other printing technologies. Examples include offset printing and inkjet and solid transfix machines.

FIG. 2A depicts the fusing configuration **300B** using a fuser belt shown in FIG. 1 in accordance with the present

teachings. The configuration **300B** can include a fuser belt of FIG. 1 that forms a fuser nip with a pressure applying mechanism **335**, such as a pressure belt, for an image supporting material **315**. In various embodiments, the pressure applying mechanism **335** can be used in combination with a heat lamp (not shown) to provide both the pressure and heat for the fusing process of the toner particles on the image supporting material **315**. In addition, the configuration **300B** can include one or more external heat rolls **350** along with, e.g., a cleaning web **360**, as shown in FIG. 2A.

FIG. 2B depicts the fusing configuration **400B** using a fuser belt shown in FIG. 1 in accordance with the present teachings. The configuration **400B** can include a fuser belt (i.e., **200** of FIG. 1) that forms a fuser nip with a pressure applying mechanism **435**, such as a pressure belt in FIG. 2B, for a media substrate **415**. In various embodiments, the pressure applying mechanism **435** can be used in a combination with a heat lamp to provide both the pressure and heat for the fusing process of the toner particles on the media substrate **415**. In addition, the configuration **400B** can include a mechanical system **445** to move the fuser belt **200** and thus fusing the toner particles and forming images on the media substrate **415**. The mechanical system **445** can include one or more rolls **445a-c**, which can also be used as heat rolls when needed.

FIG. 3 demonstrates a view of an embodiment of a transfix member **7** which may be in the form of a belt, sheet, film, or like form. The transfix member **7** is constructed similarly to the fuser belt described above. The developed image **12** positioned on intermediate transfer member **1**, is brought into contact with and transferred to transfix member **7** via rollers **4** and **8**. Roller **4** and/or roller **8** may or may not have heat associated therewith. Transfix member **7** proceeds in the direction of arrow **13**. The developed image is transferred and fused to a copy substrate **9** as copy substrate **9** is advanced between rollers **10** and **11**. Rollers **10** and/or **11** may or may not have heat associated therewith.

Described herein is a polyimide composition suitable for use as a substrate layer **210** of FIG. 1. The polyimide composition includes an internal release agent that self releases from a metal substrate such as stainless steel. Most references report applying an external release layer on the metal substrate before coating the polyimide layer, and then releasing it. The disclosed composition is cost effective since only one coating layer is needed.

#### Substrate Layer

The substrate layer **210** disclosed herein is a polyimide composition comprising an internal release agent of a fluoro acid, that self releases from a metal substrate such as stainless steel. The prior art teaches applying an external release layer on the metal substrate before coating the polyimide layer, and then releasing it. The disclosed composition is cost effective since only one coating layer is needed.

In an embodiment, the disclosed composition comprises a polyamic acid such as a polyamic acid of biphenyl tetracarboxylic dianhydride/4,4'-oxydianiline and an internal release agent such as a dodecafluorosuberic acid, where the dodecafluorosuberic acid can chemically interact with the polyamic acid, and thus be incorporated into the polyimide network instead of physical blending. The amount of the release agent is from about 0.1 weight percent to about 5.0 weight percent of the substrate.

Certain liquid fluoro agents are used as releasing agents such as perfluoropolyethers. However, when mixed with a polyamic acid, they are incompatible with the polyamic acid coating solution (phase separation), and the resulting polyimide shows clear phase separation. The releasing of the

polyimide from the coating substrate varies and is very difficult to control with such liquid fluoro agents.

The disclosed polyamic acid includes one of a polyamic acid of pyromellitic dianhydride/4,4'-oxydianiline, a polyamic acid of pyromellitic dianhydride/phenylenediamine, a polyamic acid of biphenyl tetracarboxylic dianhydride/4,4'-oxydianiline, a polyamic acid of biphenyl tetracarboxylic dianhydride/phenylenediamine, a polyamic acid of benzophenone tetracarboxylic dianhydride/4,4'-oxydianiline, a polyamic acid of benzophenone tetracarboxylic dianhydride/4,4'-oxydianiline/phenylenediamine, and the like and mixtures thereof.

Commercial examples of polyamic acid of pyromellitic dianhydride/4,4'-oxydianiline include PYRE-ML RC5019 (about 15-16 weight percent in N-methyl-2-pyrrolidone, NMP), RC5057 (about 14.5-15.5 weight percent in NMP/aromatic hydrocarbon=80/20), and RC5083 (about 18-19 weight percent in NMP/DMAC=15/85), all from Industrial Summit Technology Corp., Parlin, N.J.; DURIMIDE® 100, commercially available from FUJIFILM Electronic Materials U.S.A., Inc.

Commercial examples of polyamic acid of biphenyl tetracarboxylic dianhydride/4,4'-oxydianiline include U-VARNISH A, and S (about 20 weight in NMP), both from UBE America Inc., New York, N.Y.

Commercial examples of polyamic acid of biphenyl tetracarboxylic dianhydride/phenylenediamine include PI-2610 (about 10.5 weight in NMP), and PI-2611 (about 13.5 weight in NMP), both from HD MicroSystems, Parlin, N.J.

Commercial examples of polyamic acid of benzophenone tetracarboxylic dianhydride/4,4'-oxydianiline include RP46, and RP50 (about 18 weight percent in NMP), both from Unitech Corp., Hampton, Va.

Commercial examples of polyamic acid of benzophenone tetracarboxylic dianhydride/4,4'-oxydianiline/phenylenediamine include PI-2525 (about 25 weight percent in NMP), PI-2574 (about 25 weight percent in NMP), PI-2555 (about 19 weight percent in NMP/aromatic hydrocarbon=80/20), and PI-2556 (about 15 weight percent in NMP/aromatic hydrocarbon/propylene glycol methyl ether=70/15/15), all from HD MicroSystems, Parlin, N.J.

Various amounts of polyamic acid can be selected for the substrate, such as for example, from about 95 to about 99.9 weight percent, from about 96 to about 99.8 weight percent, or from about 97 to about 99.5 weight percent.

Other polyamic acid or ester of polyamic acid examples that can be included in the intermediate transfer member are from the reaction of a dianhydride and a diamine. Suitable dianhydrides include aromatic dianhydrides and aromatic tetracarboxylic acid dianhydrides such as, for example, 9,9-bis(trifluoromethyl)xanthene-2,3,6,7-tetracarboxylic acid dianhydride, 2,2-bis(3,4-dicarboxyphenyl)hexafluoropropane dianhydride, 2,2-bis((3,4-dicarboxyphenoxy)phenyl)hexafluoropropane dianhydride, 4,4'-bis(3,4-dicarboxy-2,5,6-trifluorophenoxy)octafluorobiphenyl dianhydride, 3,3',4,4'-tetracarboxybiphenyl dianhydride, 3,3',4,4'-tetracarboxybenzophenone dianhydride, di-(4-(3,4-dicarboxyphenoxy)phenyl)ether dianhydride, di-(4-(3,4-dicarboxyphenoxy)phenyl) sulfide dianhydride, di-(3,4-dicarboxyphenyl)methane dianhydride, di-(3,4-dicarboxyphenyl)ether dianhydride, 1,2,4,5-tetracarboxybenzene dianhydride, 1,2,4-tricarboxybenzene dianhydride, butanetetracarboxylic dianhydride, cyclopentanetetracarboxylic dianhydride, pyromellitic dianhydride, 1,2,3,4-benzenetetracarboxylic dianhydride, 2,3,6,7-naphthalenetetracarboxylic dianhydride, 1,4,5,8-naphthalenetetracarboxylic dianhydride, 1,2,5,6-naphthalenetetracarboxy-

lic dianhydride, 3,4,9,10-perylenetetracarboxylic dianhydride, 2,3,6,7-anthracene tetracarboxylic dianhydride, 1,2,7,8-phenanthrenetetracarboxylic dianhydride, 3,3',4,4'-biphenyltetracarboxylic dianhydride, 2,2',3,3'-biphenyltetracarboxylic dianhydride, 3,3',4-4'-benzophenonetetracarboxylic dianhydride, 2,2',3,3'-benzophenonetetracarboxylic dianhydride, 2,2-bis(3,4-dicarboxyphenyl)propane dianhydride, 2,2-bis(2,3-dicarboxyphenyl)propane dianhydride, bis(3,4-dicarboxyphenyl)ether dianhydride, bis(2,3-dicarboxyphenyl)ether dianhydride, bis(3,4-dicarboxyphenyl)sulfone dianhydride, bis(2,3-dicarboxyphenyl)sulfone 2,2-bis(3,4-dicarboxyphenyl)-1,1,1,3,3,3-hexafluoropropane dianhydride, 2,2-bis(3,4-dicarboxyphenyl)-1,1,1,3,3,3-hexachloropropane dianhydride, 1,1-bis(2,3-dicarboxyphenyl)ethane dianhydride, 1,1-bis(3,4-dicarboxyphenyl)ethane dianhydride, bis(2,3-dicarboxyphenyl)methane dianhydride, bis(3,4-dicarboxyphenyl)methane dianhydride, 4,4'-(p-phenylenedioxy)diphthalic dianhydride, 4,4'-(m-phenylenedioxy)diphthalic dianhydride, 4,4'-diphenylsulfidedioxybis(4-phthalic acid)dianhydride, 4,4'-diphenylsulfonedioxybis(4-phthalic acid)dianhydride, methylenebis(4-phenyleneoxy-4-phthalic acid)dianhydride, ethylenebis(4-phenyleneoxy-4-phthalic acid)dianhydride, isopropylidenebis(4-phenyleneoxy-4-phthalic acid)dianhydride, hexafluoroisopropylidenebis(4-phenyleneoxy-4-phthalic acid)dianhydride, and the like. Exemplary diamines suitable for use in the preparation of the polyamic acid include 4,4'-bis-(m-aminophenoxy)-biphenyl, 4,4'-bis-(m-aminophenoxy)-diphenyl sulfide, 4,4'-bis-(m-aminophenoxy)-diphenyl sulfone, 4,4'-bis-(p-aminophenoxy)-diphenyl sulfide, 4,4'-bis-(p-aminophenoxy)-diphenyl sulfone, 4,4'-diamino-azobenzene, 4,4'-diaminobiphenyl, 4,4'-diaminodiphenylsulfone, 4,4'-diamino-p-terphenyl, 1,3-bis-(gamma-aminopropyl)-tetramethyl-disiloxane, 1,6-diaminohexane, 4,4'-diaminodiphenylmethane, 3,3'-diaminodiphenylmethane, 1,3-diaminobenzene, 4,4'-diaminodiphenyl ether, 2,4'-diaminodiphenylether, 3,3'-diaminodiphenylether, 3,4'-diaminodiphenylether, 1,4-diaminobenzene, 4,4'-diamino-2,2',3,3',5,5',6,6'-octafluoro-biphenyl, 4,4'-diamino-2,2',3,3',5,5',6,6'-octafluorodiphenyl ether, bis[4-(3-aminophenoxy)phenyl]sulfide, bis[4-(3-aminophenoxy)phenyl]sulfone, bis[4-(3-aminophenoxy)phenyl]ketone, 4,4'-bis(3-aminophenoxy)biphenyl, 2,2-bis[4-(3-aminophenoxy)phenyl]-propane, 2,2-bis[4-(3-aminophenoxy)phenyl]-1,1,3,3,3-hexafluoropropane, 4,4'-diaminodiphenyl sulfide, 4,4'-diaminodiphenyl ether, 4,4'-diaminodiphenyl sulfone, 4,4'-diaminodiphenylmethane, 1,1-di(p-aminophenyl)ethane, 2,2-di(p-aminophenyl)propane, and 2,2-di(p-aminophenyl)-1,1,1,3,3,3-hexafluoropropane, and the like and mixtures thereof.

The dianhydrides and diamines are, for example, selected in a weight ratio of from about 20:80 to about 80:20, and more specifically, in an about 50:50 weight ratio. The above aromatic dianhydride like aromatic tetracarboxylic acid dianhydrides and diamines like aromatic diamines are used singly or as a mixture, respectively.

The release agent as the internal release agent includes a fluoro acid of the formula  $\text{HOOC}(\text{CF}_2)_n\text{COOH}$  or  $\text{C}_n\text{F}_{2n+1}\text{COOH}$ , where  $n$  is from 2 to 18, or from 2 to 12, or from 2 to 10. Embodiments of the fluoro acid include octafluorosuberic acid  $\text{HOOC}(\text{CF}_2)_4\text{COOH}$ , dodecafluorosuberic acid  $\text{HOOC}(\text{CF}_2)_6\text{COOH}$ , hexadecafluorosebacic acid  $\text{HOOC}(\text{CF}_2)_8\text{COOH}$ , heptadecafluoro-n-nonanoic acid  $\text{CF}_3(\text{CF}_2)_7\text{COOH}$ , nonadecafluorodecanoic acid  $\text{CF}_3(\text{CF}_2)_8\text{COOH}$ , nonafluorovaleric acid  $\text{CF}_3(\text{CF}_2)_3\text{COOH}$ , pentadecafluorooctanoic

acid  $\text{CF}_3(\text{CF}_2)_6\text{COOH}$ , and undecafluorohexanoic acid  $\text{CF}_3(\text{CF}_2)_4\text{COOH}$ , and the like and mixtures thereof.

The release agent disclosed herein is compatible with the coating solution (clear when mixed), and the resulting polyimide is also clear with no apparent phase separation. In addition, the fluoro acid can chemically interact with the polyamic acid, and thus be incorporated into the polyimide network instead of physical blending. The resulting polyimide self releases from the metal coating substrate.

Various amounts of fluoro acid can be selected for the substrate, such as for example, from about 0.1 to about 5 weight percent of the substrate, from about 0.2 to about 4 weight percent, or from about 0.5 to about 3 weight percent of the substrate.

The polyimide substrate composition can optionally contain a polysiloxane copolymer to enhance or smooth the coating. The concentration of the polysiloxane copolymer is less than about 1 weight percent or less than about 0.2 weight percent. The optional polysiloxane copolymer includes a polyester modified polydimethylsiloxane, commercially available from BYK Chemical with the trade name of BYK® 310 (about 25 weight percent in xylene) and 370 (about 25 weight percent in xylene/alkylbenzenes/cyclohexanone/monophenylglycol=75/11/7/7); a polyether modified polydimethylsiloxane, commercially available from BYK Chemical with the trade name of BYK® 330 (about 51 weight percent in methoxypropylacetate) and 344 (about 52.3 weight percent in xylene/isobutanol=80/20), BYK®-SILCLEAN 3710 and 3720 (about 25 weight percent in methoxypropanol); a polyacrylate modified polydimethylsiloxane, commercially available from BYK Chemical with the trade name of BYK®-SILCLEAN 3700 (about 25 weight percent in methoxypropylacetate); or a polyester polyether modified polydimethylsiloxane, commercially available from BYK Chemical with the trade name of BYK® 375 (about 25 weight percent in Di-propylene glycol monomethyl ether). The polyimide, the fluoro acid and the polysiloxane polymer of the substrate are present in a weight ratio of about 99.9/0.09/0.01 to about 95/4/1.

The disclosed polyimide substrate layer 210 possesses a Young's modulus of from about 4,000 MPa to about 10,000 MPa, or from about 5,000 MPa to about 10,000 MPa, or from about 6,000 MPa to about 10,000 MPa; and an onset decomposition temperature of from about 400° C. to about 600° C., or from about 425° C. to about 575° C., or from about 450° C. to about 550° C.

Also described herein is a composition used in a process of preparing a seamless polyimide belt for a fuser belt substrate via flow coating. In a centrifugal molding process, a thin fluorine or silicone release layer is applied on the inside of a rigid cylindrical mandrel, and then the polyimide layer is applied and subsequently cured and released from the mandrel. Using a flow coating process and the disclosed composition eliminates the requirement of an extra release layer, thus reducing manufacturing cost.

The composition of the substrate layer comprises a polyamic acid such as a polyamic acid of pyromellitic dianhydride/4,4-oxydianiline and an internal release agent of a fluoro acid. The internal release agent is present in an amount of from about 0.05 weight percent to about 0.5 weight percent or from about 0.1 weight percent to about 0.4 weight percent or from about 0.15 weight percent to about 0.3 weight percent of the substrate. The fluoro acid release agent is needed to fully release the polyimide layer from the stainless steel substrate.

The polyimide-fluoro acid composition is flow coated on a welded stainless steel belt or an electroformed seamless nickel belt at the desired product circumference. The polyimide-fluoro acid belt is partially cured, or pre-cured, at from about 150° C. to about 250° C., or from about 180° C. to about 220° C. for a time of from about 30 minutes to about 90 minutes, or from about 45 minutes to about 75 minutes, and self releases from the stainless steel belt or electroformed seamless nickel belt, and then is further completely cured at from about 250° C. to about 370° C., or from about 300° C. to about 340° C., for a time of from about 30 minutes to about 150 minutes, or from about 60 minutes to about 120 minutes under tension in the configuration shown in FIG. 4. This final curing is at a tension of from about 1 kilogram to about 10 kilograms. As shown in FIG. 4, the pre-cured belt 410 is tensioned between two rollers 250 while rotating the direction of arrow 20. The final curing produces a belt that exhibits a modulus suitable for use as a fuser member.

The seam thickness and profile of the seamed stainless steel belt can be minimized, and the surface finish and roughness of the substrate belt can be specified. For example, a rough lathed or honed belt is better for the polyimide layer release. Such a configuration easily allows the production of belts of various lengths and widths. Using a rotating mandrel limits the width and length of the belts able to be produced as each belt requires a separate mandrel.

In one embodiment, the coating belt substrate is a rough lathed belt substrate with a  $R_a$  (average roughness) of from about 0.01 micron to about 0.5 micron, or from about 0.05 micron to about 0.3 micron, or from about 0.1 micron to about 0.2 micron; and a  $R_{max}$  or from about 0.05 micron to about 2 micron, or from about 0.1 micron to about 1 micron, or from about 0.2 micron to about 0.7 micron. The back of the polyimide fuser substrate flow coated from this substrate is similarly rough lathed, thus recognizable.

In another embodiment, the coating belt substrate is a honed belt substrate with a  $R_a$  of from about 0.15 micron to about 1 micron, or from about 0.2 micron to about 0.8 micron, or from about 0.3 micron to about 0.7 micron; and a  $R_{max}$  of from about 0.5 micron to about 10 microns, or from about 1 micron to about 7 microns, or from about 2 microns to about 4 microns. The back of the polyimide fuser substrate flow coated from this substrate is similarly honed, thus recognizable.

The polyimide-fluoro acid layer thickness can be achieved by single pass or multi pass coating. For single pass, the polyimide layer is coated, and pre-cured at a temperature between about 125° C. and about 250° C. for a time of about 30 minutes to about 90 minutes, and then fully cured at a temperature between about 250° C. and about 370° C. for a time of about 30 minutes to about 90 minutes. For multi-pass, such as dual pass, the bottom polyimide layer is coated on a substrate and pre-cured between about 125° C. and about 190° C. for a time of about 30 minutes to about 90 minutes, and the top polyimide layer is subsequently coated and pre-cured between about 125° C. and about 190° C. for a time of about 30 minutes to about 90 minutes, and then the dual layer polyimide layer is fully cured at a temperature between about 190° C. and about 370° C. for a time of about 30 minutes to about 90 minutes. In an embodiment a stainless steel belt is used as the coating substrate. The substrate is rotated at a speed of from about 20 rpm to about 100 rpm, or from about 40 rpm to about 60 rpm during the thermal curing of the coating.

The polyimide substrate composition includes a solvent. Examples of the solvent selected to form the composition include toluene, hexane, cyclohexane, heptane, tetrahydrofu-

ran, methyl ethyl ketone, methyl isobutyl ketone, N,N'-dimethylformamide, N,N'-dimethylacetamide, N-methylpyrrolidone (NMP), methylene chloride and the like and mixtures thereof where the solvent is selected, for example, in an amount of from about 70 weight percent to about 95 weight percent, and from 80 weight percent to about 90 weight percent based on the amounts in the coating mixture.

Additives and additional conductive or non-conductive fillers may be present in the above-described composition. In 10 various embodiments, other filler materials or additives including, for example, inorganic particles, can be used for the coating composition and the subsequently formed surface layer. Fillers used herein include carbon blacks such aluminum nitride, boron nitride, aluminum oxide, graphite, 15 graphene, copper flake, nano diamond, carbon black, carbon nanotube, metal oxides, doped metal oxide, metal flake, and mixtures thereof. In various embodiments, other additives known to one of ordinary skill in the art can also be included to form the disclosed composite materials.

20 The composition is coated on a substrate in any suitable known manner. Typical techniques for coating such materials on the substrate layer include flow coating, liquid spray coating, dip coating, wire wound rod coating, fluidized bed coating, powder coating, electrostatic spraying, sonic spraying, blade coating, molding, laminating, and the like.

25 Specific embodiments will now be described in detail. These examples are intended to be illustrative, and not limited to the materials, conditions, or process parameters set forth in these embodiments. All parts are percentages by solid weight unless otherwise indicated.

## EXAMPLES

30 A composition comprising polyamic acid of biphenyl tetra-carboxylic dianhydride/4,4'-oxydianiline and dodecafluorosuberic acid in a weight ratio of about 99.5 to 0.5 was prepared in N-methylpyrrolidone (NMP), at about 16 solid weight percent. The polyamic acid is from Kaneka Corp.; and dodecafluorosuberic acid is from TCI America. The composition liquid was coated on a stainless steel substrate, and subsequently cured at 75° C. for 30 minutes, 190° C. for 30 minutes and 320° C. for 60 minutes. The resulting polyimide fuser belt self released from the stainless steel substrate, and an 80  $\mu$ m smooth polyimide substrate was obtained.

35 The polyimide/dodecafluorosuberic acid substrate was further tested for modulus and coefficient of thermal expansion (CTE). The Young's modulus was about 7,100 MPa, and the CTE was 17 ppm/ $^{\circ}$  K. As a comparison, a commercially available polyimide belt's (Nitto Denko KUC polyimide) modulus was about 6,000 MPa, and the CTE was 15 ppm/ $^{\circ}$  K.

40 The onset decomposition temperature of the disclosed polyimide/dodecafluorosuberic acid substrate was about 590° C. As a comparison, the onset decomposition temperature of the Nitto Denko KUC polyimide substrate was about 510° C.

45 Thus, the key properties of the disclosed polyimide/dodecafluorosuberic acid fuser belt substrate were comparable to those of commercially available polyimide substrates, however with lower manufacturing cost due to elimination of the extra release layer coating.

50 It will be appreciated that variants of the above-disclosed and other features and functions or alternatives thereof may be combined into other different systems or applications. Various presently unforeseen or unanticipated alternatives, modifications, variations, or improvements therein may be subsequently made by those skilled in the art, which are also encompassed by the following claims.

## 11

What is claimed is:

1. A fuser member comprising:  
a substrate layer comprising a polyimide polymer and a  
fluoro acid, wherein the fluoro acid is selected from the  
group consisting of:  $\text{HOOC}(\text{CF}_2)_n\text{COOH}$  and  $\text{C}_n\text{F}_{2n+1}$   
 $\text{COOH}$ , wherein n is from 2 to 18.

2. The fuser member of claim 1 wherein the substrate layer  
further comprises a polysiloxane polymer.

3. The fuser member of claim 2 wherein the polysiloxane  
polymer is selected from the group consisting of a polyester  
modified polydimethylsiloxane, a polyether modified poly-  
dimethylsiloxane, a polyacrylate modified polydimethylsil-  
oxane, and a polyester polyether modified polydimethylsil-  
oxane.

4. The fuser member of claim 1 wherein the polyimide  
polymer and the fluoro acid are present in a weight ratio of  
about 99.9/0.1 to about 95/5.

5. The fuser member of claim 1 wherein the substrate layer  
comprises a modulus of from about 4000 MPa to about  
10,000 MPa.

6. The fuser member of claim 1 wherein the substrate layer  
further comprises fillers.

7. The fuser member of claim 6 wherein the fillers are  
selected from the group consisting of aluminum nitride,  
boron nitride, aluminum oxide, graphite, graphene, copper  
flake, nano diamond, carbon black, carbon nanotube, metal  
oxides, doped metal oxide, metal flake, and mixtures thereof.

8. The fuser member of claim 1 further comprising:  
an intermediate layer disposed on the substrate layer; and  
a release layer disposed on the intermediate layer.

9. The fuser member of claim 8 wherein the intermediate  
layer comprises silicone.

10. The fuser member of claim 8 further wherein the  
release layer comprises a fluoropolymer.

11. A fuser member comprising:  
a substrate layer comprising a polyimide polymer and a  
fluoro acid selected from the group consisting of  $\text{HOOC}$   
 $(\text{CF}_2)_n\text{COOH}$  and  $\text{C}_n\text{F}_{2n+1}\text{COOH}$ , wherein n is from 2  
to 18;

## 12

an intermediate layer disposed on the substrate layer, com-  
prising a material selected from the group consisting of  
silicone and fluoroelastomer; and

a release layer disposed on the intermediate layer comprising  
a fluoropolymer wherein the substrate layer has a  
modulus of from about 4,000 MPa to about 10,000 MPa.

12. The fuser member of claim 11 wherein the release layer  
further comprises fillers.

13. The fuser member of claim 12 wherein the fillers are  
selected from the group consisting of aluminum nitride,  
boron nitride, aluminum oxide, graphite, graphene, copper  
flake, nano diamond, carbon black, carbon nanotube, metal  
oxides, doped metal oxide, metal flake, and mixtures thereof;  
and wherein the fluoropolymer comprises a fluoroelastomer  
or a fluoroplastic.

14. The fuser member of claim 11 further comprising:  
an adhesive layer disposed on the intermediate layer or the  
substrate layer.

15. The fuser member of claim 11, wherein the fluoro acid  
comprises dodecafluorosuberic acid.

16. A fuser member comprising:  
a substrate layer comprising a polyimide polymer and a  
fluoro acid selected from the group consisting of  $\text{HOOC}$   
 $(\text{CF}_2)_n\text{COOH}$  and  $\text{C}_n\text{F}_{2n+1}\text{COOH}$ , wherein n is from 2  
to 18, the substrate layer comprising a modulus of from  
about 4,000 MPa to about 10,000 MPa and an onset  
decomposition temperature of about 590° C.

17. The fuser member of claim 16 further comprising:  
an intermediate layer disposed on the substrate layer; and  
a release layer disposed on the intermediate layer.

18. The fuser member of claim 16 wherein the intermediate  
layer comprises silicone.

19. The fuser member of claim 16 further wherein the  
release layer comprises a fluoropolymer.

\* \* \* \* \*